

# UNITED STATES PATENT OFFICE.

ALBRECHT SCHMIDT, OF HÖCHST-ON-THE-MAIN, GERMANY, ASSIGNOR TO FARBWERKE VORM. MEISTER LUCIUS & BRÜNING, OF HÖCHST-ON-THE-MAIN, GERMANY, A CORPORATION OF GERMANY.

## UNEXPLOSIVE PREPARATION.

1,136,723.

Specification of Letters Patent.

Patented Apr. 20, 1915.

No Drawing.

Application filed September 28, 1913. Serial No. 792,465.

To all whom it may concern:

Be it known that I, ALBRECHT SCHMIDT, Ph.D., chemist, a citizen of the Empire of Germany, residing at Höchst-on-the-Main, 5 Germany, have invented certain new and useful Improvements in Unexplosive Preparations, of which the following is a specification.

It is known that nitro compounds, for instance salts of dinitro-and polynitro-phenols, such as sodium-dinitro-cresolate, sodium-dinitro-phenolate or the like, are used for several purposes, serving also as mycocide substances. The use *i. e.* the handling 10 of these products in the trade, above all for over-sea-transport, appears to involve some danger inasmuch as the pastes therefrom, when dry, leave behind certain bodies which are of an exceedingly explosive action. 15 Thus it is a well-known fact that salts of dinitrophenols, for instance, 1,2,4-sodium-dinitro-phenolate, also sodium-dinitro-cresolate and the trinitro compounds, are very explosive, so that it is dangerous to store 20 and move the highly concentrated pastes of these salts in places which are not fire-proof, because when a fire breaks out said pastes dry up very quickly and then explode.

Now I have found that the explosiveness 25 of such bodies can be subdued in a most simple and inexpensive way by mixing these bodies with the constituents of waste liquors from sulfite-cellulose or with the latter itself (both to be comprised under the term 30 "waste liquors from sulfite-cellulose"). By "constituents" of waste liquors from sulfite-cellulose are to be understood salts of ligninic acids or lignino-sulfonates or the like. In this way, that is to say by evaporating 35 such pastes, it is possible to obtain unexplosive solid products. Thus for instance a paste is produced, which is capable of being transported and which, even when artificially and completely dried up, is no longer 40 explosive, by mixing sodium-dinitro-phenolate or the sodium-dinitro-phenolate containing common salt (as obtainable by treating dinitrochlorobenzene with caustic soda-lye) with about the same or one and a half 45 times the quantity or less of waste-liquor from sulfite-cellulose of about 80 per cent. (that is, containing about 20 per cent. of water), with or without the addition of a 50

further quantity of caustic soda-lye, sodium carbonate or the like. By allowing the 55 pastes thus obtained to dry at a moderately high temperature, for instance *in vacuo*, solid products are obtained, which, even when suddenly heated, do not explode but only glow faintly. In cases where it is not 60 intended to suppress entirely the explosiveness of nitro-bodies but only to diminish it, considerably less of the ligninosulfonate is added.

The waste-liquor from sulfite-cellulose 65 possesses, probably owing to its caking and sticky condition, the property of lessening the mobility of the individual particles of the respective explosive body, and consequently the transmissibility of the ignition 70 of such a particle to another one.

The pastes thus obtained for instance from the salts of dinitrophenols are also distinguished by their ready solubility, furthermore they dry up very slowly, a property which is also of great importance for the sale of the product in cheap packages. Finally the pastes are entirely stable, the 75 ligninosulfonates having proved to be indifferent toward nitro-bodies at ordinary temperature or at a slightly-raised temperature.

The above described process can be applied to all nitro-bodies, among which are also introduced nitrosulfonic acids or the like.

Having now described my invention, what I claim is:

1. As new products, the preparations, obtained by incorporating waste-liquors from sulfite-cellulose into nitro compounds, showing on the one hand the reactions of the waste-liquors from sulfite-cellulose, on the other hand, those of the nitro compounds.

2. As a new product, the preparation, obtained by incorporating the waste-liquors from sulfite-cellulose into the alkali salt of the dinitrophenol, showing on the one hand the reactions of the waste-liquors from sulfite-cellulose, on the other hand, those of the dinitrophenol.

In testimony whereof I affix my signature in presence of two witnesses.

ALBRECHT SCHMIDT.

Witnesses:

JEAN GRUND,  
CARL GRUND.